

## UNITED STATES PATENT OFFICE

2,613,179

## SILVER PLATING

Henry Wölfsön and Bernard Thomson, London, England, assignors to International Standard Electric Corporation, New York, N. Y.

No. Drawing. Application June 19, 1947; Serial No. 755,738. In Great Britain June 20, 1946.

8 Claims. (Cl. 204—46)

1

This invention relates to electrolytes for silver plating and to silver plating baths and has for its object to provide an electrolyte and bath capable of producing excellent bright deposits at high current densities.

The use of potassium nitrate has been previously advocated by Promisel and Wood: Trans. Electrochemical Society, 1941; and it was claimed that the addition of this salt to a silver cyanide bath has a beneficial effect on the operation of the bath and on the appearance of the plate. Experiments we have made substantiated these claims, semi-bright deposits being obtained from plating solutions containing 100—150 gm. per litre of potassium nitrate at current densities up to about 30 amp./ft.<sup>2</sup>.

The maximum current density at which a conventional bath could be satisfactorily worked under similar conditions was about 18 amp./ft.<sup>2</sup>.

An article by R. Weiner in Metallwirtschaft 22, 472-4, 1943, claims that bright silver deposits are obtained at current densities of 18-27 a./ft.<sup>2</sup> from a solution the essential feature of which is the addition of selenium (as selenite) to a cyanide bath containing about 40 gm. per litre of silver. Experiments we have carried out show these claims to be, in the main, justified. At an optimum concentration of potassium selenite of 0.5-1.5 g./l. (equivalent to 0.2-0.6 gm. of selenium per litre), selenium had a marked effect on the plate and semi-bright deposits of good quality were obtained at current densities up to 28 amp./ft.<sup>2</sup>.

Further experiments have led to the surprising discovery that the two addition agents selenium and potassium nitrate are, together, very much more potent than either individually. It is the use of the two in combination which is the distinctive and novel feature of an electrolyte, from which we are able to produce excellent bright deposits of silver at current densities some four to six times greater than could be used with a conventional plating solution.

The formulae for our preferred solutions were evolved after a number of experiments aimed at determining the most useful concentration of the two addition agents. We varied the potassium nitrate content of the baths between 25 and 200 grams per litre and found a concentration of 100-150 g./l. to be most effective. Potassium selenite was added in stages corresponding to a selenium content of from 0.015 to 1.0 g./l., and the range 0.2-0.6 g./l. was shown to be the most favourable.

The concentration of the other constituents of

2

the electrolyte does not seem to be critical. Most of our work was done with solutions containing 40 g./l. of silver cyanide but we believe quite wide variations from this figure could be tolerated. It seems necessary (at least while working at the higher current densities) to maintain the customary fairly high concentration of "free cyanide." Most silver plating solutions contain an appreciable quantity of potassium carbonate, but we prefer not to include this salt as it appears to diminish the beneficial effect of the potassium nitrate on selenium.

The invention is not necessarily limited to the addition of selenium as selenite, other soluble selenium salts may be found to be suitable.

Our preferred solutions and the recommended working conditions are as follows:

|                    | Electrolyte A         | Electrolyte B |
|--------------------|-----------------------|---------------|
| Silver cyanide     | g./l.                 | 40            |
| Potassium cyanide  | g./l.                 | 55            |
| Potassium nitrate  | g./l.                 | 100           |
| Potassium selenite | g./l.                 | 1.0           |
| Current density    | amp./ft. <sup>2</sup> | 20-75         |
|                    |                       | 20-100        |

Room temperature: Moderate agitation.  
Anodes—silver, two to four times area of cathode, or more.

Electrolyte A appears to yield a deposit of slightly superior quality to Electrolyte B; on the other hand Electrolyte B has a rather wider range of current density.

The ratio between the areas of the anode and cathode of a bath using an electrolyte according to the invention should be greater than that normally accepted, as otherwise anode dissolution might be impaired at the high current densities employed.

Sodium salts or other alkali metal salts may be used wholly or partly in place of potassium salts on an equivalent basis.

Substantial increase of speed of deposition can be obtained with a stationary cathode and without any form of agitation of the solution, an anode having an area about twice that of the cathode, and a current density of the order of 10 amp./ft.<sup>2</sup>, but the full advantage of the invention requires a rocking or like cathode and/or other method of agitation but of course without aeration, and higher current densities. With current densities above 20 amp./ft.<sup>2</sup>, an anode up to four times the area of the cathode or more will be required.

By the use of the invention not only is the speed of operation increased but the bright finish obtained substantially reduces or eliminates the

additional processes required such as scratch brushing, and the surface is much more responsive to buffing.

We claim:

1. An argentocyanide electrolyte for use in electrodepositing bright silver plate at high current densities of at least 10 amp./ft.<sup>2</sup> of cathode area that consists essentially of an aqueous solution of the following substances in substantially the proportions indicated:

|                    | G./L |
|--------------------|------|
| Silver cyanide     | 40   |
| Potassium cyanide  | 55   |
| Potassium nitrate  | 100  |
| Potassium selenite | 1.0  |

2. An argentocyanide electrolyte for use in electrodepositing bright silver plate at high current densities of at least 10 amp./ft.<sup>2</sup> of cathode area, that consists essentially of an aqueous solution of the following substances in substantially the proportions indicated:

|                    | G./L |
|--------------------|------|
| Silver cyanide     | 40   |
| Potassium cyanide  | 55   |
| Potassium nitrate  | 150  |
| Potassium selenite | 1.0  |

3. An argentocyanide electrolyte for use in electrodepositing bright silver plate at high current densities of at least 10 amp./ft.<sup>2</sup> of cathode area that consists essentially of an aqueous solution of the following substances in substantially the proportions indicated:

|                       | G./L    |
|-----------------------|---------|
| Silver cyanide        | 40      |
| Potassium cyanide     | 55      |
| Alkali metal nitrate  | 100-150 |
| Alkali metal selenite | 0.5-1.5 |

4. An argentocyanide electrolyte according to claim 3 in which the alkali metal nitrate is potassium nitrate and the alkali metal selenite is potassium selenite.

5. A process for electrodepositing a bright silver

plate upon an article that comprises making the article the cathode during electrolysis at a current density of at least 10 amp./ft.<sup>2</sup> of cathode area, of an electrolyte that consists essentially of an aqueous solution of the following substances in substantially the indicated proportions.

|                       | G./L    |
|-----------------------|---------|
| Silver cyanide        | 40      |
| Potassium cyanide     | 55      |
| Alkali metal nitrate  | 100-150 |
| Alkali metal selenite | 0.5-1.5 |

6. A process according to claim 5 in which the alkali metal nitrate is potassium nitrate and the alkali metal selenite is potassium selenite.

7. A process according to claim 6 in which the potassium nitrate is present in the amount of 100 g./l. and the potassium selenite in the amount of 1.0 g./l.

8. A process according to claim 6 in which the potassium nitrate is present in the amount of 150 g./l. and the potassium selenite in the amount of 1 g./l.

HENRY WOLFSON.  
BERNARD THOMSON.

#### REFERENCES CITED

The following references are of record in the file of this patent:

#### UNITED STATES PATENTS

| Number    | Name    | Date           |
|-----------|---------|----------------|
| 2,440,672 | Green   | May 4, 1948    |
| 2,449,726 | Slatkin | Sept. 21, 1948 |

#### OTHER REFERENCES

Egeberg et al.: Transactions of the Electrochemical Society, vol. 74 (1938), pages 211-227.

Modern Electroplating, published 1942 by the American Electrochemical Society, pages 290, 291.

Metallwirtschaft, vol. 22, (1943), pages 472 to

474, an article by Weiner.

Ser. No. 351,241, Weiner (A. P. C.), published

May 18, 1943.